

Dec. 21, 1965

J. G. TEMPLETON

3,224,123

LABEL FOR HOSIERY

Filed Nov. 5, 1962



FIG. 1.



FIG. 2.

INVENTOR  
JOHN G. TEMPLETON

BY *Drice & Hennefeld*

ATTORNEYS

## 1

3,224,123

## LABEL FOR HOSIERY

John G. Templeton, Grand Rapids, Mich., assignor to  
Rose Patch & Label Company, Grand Rapids, Mich.,  
a corporation of Michigan

Filed Nov. 5, 1962, Ser. No. 235,243  
5 Claims. (Cl. 40—2)

This invention concerns textile labels, and more particularly labels especially adapted for the labeling of thin, stretchable knitted fabrics such as nylon stockings.

The labeling of sheer women's stockings has long presented vexing problems to the hosiery manufacturers. Due to the extreme elasticity of the stocking fabric and its extreme delicacy, it has been impossible to label such hosiery in the manner used on heavier and more sturdy fabrics, such as sewing, for example. As a result, brand designations have so far either been knitted into the welt fabric during manufacture of the stocking—an expensive method—or imprinted on the completed stocking—an unsatisfactory method because the print washes off. It will be seen that fabric strip labels would be highly desirable in the manufacture of stockings, but so far all attempts to satisfactorily and economically label nylon stockings with fabric strip labels have failed.

It has previously been proposed in the shirt labeling art to use a woven label strip and to weave into the strip on the front side thereof a series of thermoplastic yarns (U.S. Patent 2,765,814). In the use of these labels, the label strip is cut where the thermoplastic yarns appear, and the ends of the individual labels thus cut are then folded under, whereupon the label is applied to the shirt fabric by heating the label and subjecting it to pressure until all of the thermoplastic yarn melts and forms a bond between the shirt fabric and the non-thermoplastic fibers of the label.

Although labels of the above-described type are useful in the environment for which they were designed, they cannot be used on sheer stockings for several reasons. First, woven labels are not as elastic and stretchable as the knitted fabric of the stocking, and the labels therefore cannot expand sufficiently when the stocking is worn. As a result, local stresses would be produced at the points of attachment of the label, and the stocking would tear in short order. Secondly, woven labels must be folded under at their ends in order to avoid raveling. (It is for this reason that the thermoplastic threads in the aforesaid patent appear on the front side of the label so that they will be underneath the label when the edges are folded over.) After folding, the thermoplastic threads have to be melted by applying heat through two layers of fabric, and controlled pinpoint melting of the threads at discrete points is difficult. This is of little consequence in the prior art, because the thermoplastic substance merely forms a fabric-to-fabric bond in the same manner as an adhesive. For this reason, however, the bonding area of the prior art labels is stiff and nonstretchable—a property which is of little consequence in shirts, but is intolerable on sheer stockings. Also, the prior art labels have to be accurately cut so that the thermoplastic fibers will appear evenly on both ends of the label and only under the fold where they will not mar the appearance of the front of the label.

## 2

The present invention solves the problems outlined above by using a knit label strip whose flexibility and stretchability approximates that of the welt to which it is to be applied. Although the label may be similar in appearance and action to the stocking fabric, it differs therefrom in the one important respect that the entire label is uniformly knit entirely or partially of thermoplastic yarn whose melting point lies well below the softening temperature of the fiber of the stocking itself. Because the ends of a knit label do not ravel, no folding of the ends is necessary. Consequently, when heat is applied to the label for bonding it to the stocking, the heat can be applied at a series of sharply defined very small discrete points. The resulting discontinuity of the bond makes the bond as a whole extremely flexible and permits the bond to be stretched lengthwise to a surprising degree. The label is thus capable of following the stretching and flexure of the stocking material to an extent sufficient to prevent discomfort to the wearer and to prevent undue stressing of the welt material. Alternatively, the sharp definition of the heat application makes possible a very thin continuous zig-zag bond, or any other pattern which may be mechanically desirable in any given application.

It is therefore the object of the invention to provide a fabric label capable of being used for the labeling of sheer women's hosiery.

It is another object of this invention to provide a knitted fabric strip label composed entirely or partially of thermoplastic yarns having a melting point lower than the softening point of the fabric to which it is to be attached.

It is still another object of this invention to provide a fabric label capable of being attached to a sheer fabric by a thermoplastic bond capable of expanding with the base fabric.

It is a further object of this invention to provide a method of affixing a thermoplastic knit label to a fabric by the judicious use of temperature gradients which permit thermal bonding of the fabric and label without breaking the thermoplastic yarn.

These and other objects of the invention will become apparent from a perusal of the following specification, taken in connection with the accompanying drawings in which:

FIG. 1 is a fragmentary elevation of a portion of a stocking with the label of this invention affixed thereto;

FIG. 2 is an enlarged, partly diagrammatic and exaggerated sectional view along lines II—II of FIG. 1, also showing the heated dies used in a preferred method of bonding the label to the stocking, and illustrating the method by which bonding is accomplished.

In FIG. 1, which shows one possible illustrative embodiment of the invention, the numeral 10 designates the welt and the numeral 12 the subwelt of an ordinary sheer stocking whose leg is shown at 14. A label 16 is thermoplasticly attached to the welt 10 by a series of small, discrete, spaced bond elements 18. The fact that the bond elements 18 are separate and discrete allows the label fabric to flex and stretch to almost any extent the stretching of the welt fabric 22 may require. A desired designation 20 would normally be affixed to the label 16 during its fabrication process before it is attached to the stocking.

FIG. 2 schematically illustrates one method by which the bond elements 18 may be formed. In FIG. 2, the layer 22 represents the yarn of the welt 10 of the stocking. Only one layer is shown for clarity, although of course the welt would normally be formed of two layers. The layer 24 in FIG. 2 represents the yarn of the label 16, whose thickness has been somewhat exaggerated for clarity in FIG. 2. In the illustration of FIG. 2, the label 16 is composed entirely of thermoplastic yarn. After the label 16 has been placed against the welt 10, the label and welt are placed between a base plate 26 and a die 28 equipped with spaced ribs 30. In a preferred embodiment of the invention, the plate 26 and die 28 are heated separately to different temperatures. The plate 26 is brought to a temperature just below the fusion point of the thermoplastic yarn 24 of the label 16. The die 28 on the other hand, is heated to a temperature below the softening point of the welt yarn 22, but well above the fusion point of the label yarn 24. The purpose of this arrangement is to maintain the yarn 24 of the label 16 lying against the plate 26 at a temperature insufficient for fusion. When the die 28 is then brought to bear against the welt, its heat is transmitted through the welt yarn 22 to the label yarn 24. As a result, the plate side of the label is held below fusion temperature, whereas the die side of the label is brought above fusion temperature. The resulting temperature gradient in the label yarn causes the die side of the label to become sufficiently melted as at 32, to permit the welt yarn 22 to be pressed into it and bonded to it by the die 28, while the plate side of the label stays cool enough to prevent the label yarn from melting entirely and breaking the mesh.

It will be understood that since the heat transfer through the fibers depends on the die pressure and the dwell time during which the die remains in position, these parameters must be so chosen as to permit just enough heat transfer to allow only partial melting of the yarn 24 as described above.

Even if some of the yarn ends from which the label 16 is knit are other than low-melting thermoplastic yarns, it is still desirable to prevent melting of the thermoplastic yarns through their entire thickness not only because of the damage to the mesh, but also because of the improved aesthetic appearance of the label.

On the other hand, the fact that using thermoplastic yarn on some of the ends from which the label is knit and non-thermoplastic yarn on the others results in a mixed fabric which retains some mechanical strength even when the thermoplastic yarn has melted, can be utilized in situations where the above-described method is not practical. For example, such a mixed knit fabric is useful when the label is to be looped over the top of the welt and affixed on both sides of the welt, or when high-frequency dielectric means are used to produce or assist in producing the fusion heat within the thermoplastic yarn itself.

As a matter of example, the following illustrative materials and parameters have been found usable in carrying out the invention:

| Article material                                             | Label material                             | Plate temp.<br>(° F.) | Die temp.<br>(° F.) | Die pressure<br>(lbs./in. <sup>2</sup> ) | Dwell time<br>(sec.) |
|--------------------------------------------------------------|--------------------------------------------|-----------------------|---------------------|------------------------------------------|----------------------|
| Nylon 66 (S.P. 460° F.)                                      | Nylon 6 (M.P. 420° F.)                     | 330                   | 440                 | 1,280                                    | 1/6                  |
| "Daeron" polyester fiber<br>(M.P. 480° F.) (S.P.<br>460° F.) | "Vicron" polyester<br>fiber (M.P. 455° F.) | 380                   | 460                 | 1,280                                    | 1/6                  |

S.P.=softening point. M.P.=melting point.

It will be appreciated that as the die temperature approaches the softening point of the article material, some weakening of the article material at the bond is prone to occur.

As a practical matter, it is preferable to use polymers of the same family for the label fiber and the article fiber, i.e. a polyamide with a polyamide, or a polyester with a polyester, because polymers of the same family generally adhere better to each other than do polymers of different families.

It should be understood that although the label 16 has been described herein as flat and attached to the welt 10, it may be equally well be miter folded or looped, or affixed to a subwelt 12 or to any other part of the article if this should appear desirable. Likewise, the bond elements 18 or corresponding pattern may run along the selvage 34 rather than along the cut edges 36, if desired. Other variations of the principles and method of the invention are of course possible, and I therefore do not desire to be limited by the embodiment shown and described, but only by the scope of the appended claims.

I claim:

1. In combination, a stretchable sheer textile article and an attached label, said article being formed of flexible, stretchable, delicate, synthetic thermoplastic polymeric fibers interengaged to form a sheer delicate article; said label being formed of thermoplastic polymeric fibers of the same family of polymers as said article fibers and having flexible and stretchable characteristics similar to said article fibers to have a like stretching and flexing capacity during normal use of said article and at least some of said label fibers being of a thermoplastic material; said label fibers having a melting point below the softening point of said article fibers; and said label being permanently secured to said article by portions of its thermoplastic fibers fusion bonded to said article fibers while remaining in an unsevered condition.

2. The combination in claim 1 wherein said label is a single unfolded layer.

3. The method of applying a permanent label to a sheer textile article comprising the steps of: providing an article formed of delicate, flexible, stretchable, synthetic fibers interengaged to form a sheer article; forming a label of interengaged fibers having flexibility and stretchability closely similar to that of said article, and at least partially of thermoplastic fibers having a melting point below the softening point of said article fibers; placing said label against said article; heating a die to a temperature above the melting point of said label fibers but below the softening point of said article fibers and pressing it against said article fibers, heating a retaining plate to a temperature below said melting point of said thermoplastic label fibers and contacting said plate against said label; partially melting said thermoplastic label fibers with said die to fuse them to said article fibers, and withdrawing said heated die before said label fibers are melted completely through and severed.

4. The method in claim 3 wherein said fusion is performed at spaced intervals along said label.

5. In combination, a stretchable sheer textile article and an attached label, said article being formed of flexible, stretchable, delicate, synthetic fibers interengaged to form a sheer delicate article; said label being formed of

fibers having flexible and stretchable characteristics similar to said article fibers to have a like stretching and flexing capacity during normal use of said article and at least some of said label fibers being of a thermoplastic mate-

rial; said label fibers having a melting point below the softening point of said article fibers; said label being permanently secured to said article by portions of its thermoplastic fibers fusion bonded to said article fibers while remaining in an unsevered condition; and said fusion bonding occurring at spaced intervals along said label to allow complete flexing of said label with said article without any appreciable contractive stress being applied to said article fibers by said label.

10

## References Cited by the Examiner

## UNITED STATES PATENTS

|           |        |           |       |
|-----------|--------|-----------|-------|
| 1,538,249 | 5/1925 | Lorenz.   |       |
| 2,604,770 | 7/1952 | Ischinger | 2—239 |
| 2,828,776 | 4/1958 | Meyer     | 40—2  |
| 2,976,628 | 3/1961 | Breslow   | 40—2  |

## FOREIGN PATENTS

853,288 11/1949 France.

EUGENE R. CAPOZIO, *Primary Examiner.*  
JEROME SCHNALL, *Examiner.*